

1

2,866,755

ESTER-BASE LUBRICANT CONTAINING  
NON-CORROSIVE EP AGENT

Raymond B. Tierney, Beacon, and Robert H. Krug, Cornwall, N. Y., assignors to The Texas Company, New York, N. Y., a corporation of Delaware

No Drawing. Application May 31, 1955  
Serial No. 512,304

9 Claims. (Cl. 252—47.5)

This invention relates to a lubricating composition which is particularly designed for lubrication of turbines used in aircraft, particularly in turbo-prop and turbo-jet planes. More particularly, this invention discloses a lubricating composition containing an EP and anti-wear additive which does not adversely affect the oxidation and corrosion properties of the lubricating composition.

Mineral oil base lubricants are not satisfactory for lubrication of turbines used in jet engines which operate over a wide temperature range and usually under severe operating conditions. Specially formulated lubricants which have thermal stability, oxidation stability, good EP and anti-wear properties and a high viscosity index are required for lubrication of turbo-jet and turbo-prop engines. The requirements for a lubricating oil for turbo-prop and turbo-jet engines are set forth in MIL-L-7808B. Up to the present time, only ester-base lubricants have met these requirements.

The lubricant composition of this invention comprises a diester or a polyester as the major component and di(o-chlorophenyl) phenyl phosphate in an amount sufficient to impart EP and anti-wear properties to said lubricant composition. The di(o-chlorophenyl) phenyl phosphate usually constitutes 0.5 to 5 weight percent of the lubricant composition and materially improves the EP and anti-wear properties of the ester-base lubricant without adversely affecting its oxidation and corrosion properties.

It is well known in the art that phosphate esters, particularly aryl phosphates and halo-substituted hydrocarbon phosphates, are EP agents. Tricresyl phosphate, tri-tri-chloropropyl phosphate and tri(p-chlorophenyl) phosphate are known to possess EP properties. Of all the aryl and halo-hydrocarbon substituted phosphates tested, di(o-chlorophenyl) phenyl phosphate is unique in its action in imparting the desired EP and anti-wear properties to an ester-base lubricant without adversely affecting its oxidation and corrosion properties. Other hydrocarbon phosphates and halo hydrocarbon substituted phosphates, even though they are closely related to di(o-chlorophenyl) phenyl phosphate in chemical constitution, were either ineffective in imparting the desired EP and anti-wear properties or seriously degraded the oxidation and corrosion properties of the ester-base lubricants. The unique action of this compound in a particular environment of an ester-base lubricant is entirely unexpected since there is no analogous action in mineral oil base lubricants.

Di(o-chlorophenyl) phenyl phosphate has the following structural formula:



2

It is recommended that this compound have a Neut. No. less than 5.0 and preferably less than 2.0 in order to formulate lubricant compositions of the desired oxidation and corrosion properties. In a copending application Serial No. 512,305, filed of even date in the names of Raymond B. Tierney and Robert H. Krug, a novel method of treating di(o-chlorophenyl) phenyl phosphate to yield a product of low Neut. No. is disclosed. The method of the copending application involves contact of the di(o-chlorophenyl) phenyl phosphate under anhydrous conditions with anhydrous alkali metal carbonate at a temperature less than 160° F.

The lubricant composition of this invention contains the di(o-chlorophenyl) phenyl phosphate in an amount sufficient to improve its EP and anti-wear properties. The desired improvement in EP and anti-wear properties is effected by use of between 0.2 and 5 weight percent of di(o-chlorophenyl) phenyl phosphate. The usual concentration of the EP additive of this invention is between 1.0 and 3.0 percent.

The most commonly used ester base is an aliphatic diester of an organic dicarboxylic acid. The dicarboxylic acid component is usually an aliphatic dicarboxylic acid containing 6 to 12 carbon atoms but glutaric acid esters and succinic acid esters may also be used. From the standpoint of cost and availability, the preferred dibasic acids are adipic acid, sebacic acid and azelaic acid. The aliphatic alcohols used to form the diesters usually contain at least 4 carbon atoms and may contain 20 or more carbon atoms.  $C_6$  to  $C_{18}$  alcohols are most commonly used. Ether alcohols such as Cellosolve and carbitol may also be used in the formation of the aliphatic diesters of organic dicarboxylic acids used as the lubricating base in the compositions of this invention.

Specific examples of the dialkyl esters of aliphatic dicarboxylic acids, which are the preferred reagents for use in the lubricant compositions of the invention, are as follows: di-2-ethylhexyl sebacate, di-2-ethylhexyl azelate, di-2-ethylhexyl adipate, dilauryl azelate, di-sec-amyl sebacate, di-2-ethylhexyl alkenylsuccinate, di-2-ethoxyethyl sebacate, di-2-(2'methoxyethoxy) ethyl sebacate, di-2-(2'ethylbutoxy) ethyl sebacate, di-2-butoxyethyl azelate, di-2-(2'butoxyethoxy) ethyl alkenylsuccinate, etc.

In addition to the aliphatic dicarboxylic acid esters described above, polyester lubricants formed by a reaction of an aliphatic dicarboxylic acid, a glycol and a mono-functional compound, which is either an aliphatic mono-hydroxy alcohol or an aliphatic monocarboxylic acid, in specified mol ratios are also employed as the synthetic lubricating base in the compositions of this invention; polyesters of this type are described in U. S. 2,628,974 on Polyester Synthetic Lubricants, which issued to R. T. Sanderson on February 17, 1953. Polyesters formed by reaction of a mixture containing specified amounts of 2-ethyl-1,3-hexanediol, sebacic acid and 2-ethylhexanol and by reaction of a mixture containing adipic acid, diethylene glycol and 2-ethylhexanoic acid illustrate this class of synthetic polyester lubricating bases.

Polyesters formed by reaction of a monocarboxylic acid and a glycol may also be used as the ester component. The acid component is usually an aliphatic acid containing at least 6 carbon atoms. The glycol component is advantageously a straight glycol such as 1,6-hexanediol, but ether glycols, such as tetraethylene glycol, may also be used.

Specific examples of the diesters of glycols are the following: di-n-decanoate of 1,4-butanediol, di-2-ethylhexanoate of 1,6-hexanediol, dilaurate of 1,4-hexanediol, dioctanoate of 1,5-pentanediol, dilaurate of tetraethylene glycol, dilaurate of triethylene glycol, dioctoate of pentaethylene glycol.

The sulfur analogs of the above-described esters are also used in the formulation of the lubricating compositions of this invention. Dithioesters are exemplified by di-2-ethylhexyl thiosebacate, di-n-octyl thioadipate and the dilaurate of 1,5-pentanedithiol; sulfur analogs of polyesters are exemplified by the reaction product of adipic acid, thioglycol and 2-ethylhexyl mercaptan.

The finished lubricant composition of this invention normally contains other well known additives which act as V. I. improvers and anti-oxidants. For example, phenothiazine, which acts as an anti-oxidant and a methacrylate polymer, which acts as a V. I. improver, are usually included in the finished lubricants and are often necessary in order to meet the rigid requirements of MIL-L-7808B. Phenothiazine, which has the formula



is a particularly effective anti-oxidant and anti-corrosive agent. Phenothiazine inhibits corrosion by preventing oxidation of the components of the lubricating composition to acidic bodies which are inherently corrosive in nature. Phenothiazine is usually present in a concentration of 0.1 to 1.5 weight percent of the lubricant composition.

Methacrylate polymers are well known V. I. improvers and pour point depressors. Polyester base lubricants, although they, per se, possess excellent V. I. and pour, usually require the presence of small concentrations of methacrylate polymers to meet the rigid requirements of MIL-L-7808B. These methacrylate polymers are usually copolymers of two or more esters of methacrylic acid and usually have a molecular weight between 10,000 and 20,000. The methacrylate esters have the following general formula:



wherein R is an aliphatic radical. Copolymers which find particular use as V. I. improvers and pour point depressants are the following: a copolymer wherein R in the above formula comprises 20% lauryl, 40% octyl and 40% cetyl; a copolymer wherein R in the above formula is 50% stearyl and 50% lauryl; a copolymer wherein R in the above formula comprises 50% lauryl and 50% octyl.

Methacrylate polymers are usually sold in the form of a concentrate comprising approximately 50% polymer and 50% carrier oil. For the lubricant compositions of this invention, it has been found advisable to use an ester-type carrier oil rather than the usual mineral base lubricating oil. The use of a methacrylate ester in an ester-type carrier oil has proven particularly effective in meeting the low temperature requirements of MIL-L-7808B.

Methacrylate polymers can constitute 1 to 20 weight percent of the composition but ordinarily are used in a concentration between 1.5 and 8 weight percent.

A Schiff's base reaction product of 1 mol of an aliphatic polyamine having two primary amino groups with 2 mols of an aromatic aldehyde having the general formula A—CH=N—R—N=CH—A, where A represents an aromatic nucleus and R is an aliphatic radical having two nitrogen atoms attached directly to different carbon atoms of the same open chain, are also sometimes incorporated in the finished lubricant. Compounds of this type which generally constitute 0.05 to 0.6 weight percent of the composition act as metal deactivators as disclosed in the Downing et al., No. 2,282,513. A preferred compound of this class, which is commercially available, is disalicylal propylenediamine which is also

known as disalicylidene-1,2-diaminopropane. This compound is sold under the trade name "DMD" by E. I. Du Pont de Nemours and Company and as "Tenamene 60" by Tennessee Eastman. Examples of other compounds of this type are the following:

Di-(2-hydroxy-3-methoxybenzal) ethylenediamine  
Di-(2-hydroxybenzal) ethylenediamine  
Di-(2-hydroxybenzal) decamethylenediamine  
Di-(2-hydroxybenzal) triethylenetetramine  
Di-(2-hydroxybenzal) hexamethylenediamine  
Di-(2-hydroxybenzal) 1:3 propylenediamine  
Dibenzal ethylenediamine  
Dibenzal hexamethylenediamine  
Dibenzal diethylenetriamine  
Dibenzal triethylenetetramine  
Disalicylal ethylenediamine

The four-ball mean Hertz load test is used as a test for screening EP and anti-wear agents. A value above 20 35 in this test is necessary in order to mark a compound of interest as an EP and anti-wear agent for polyester base lubricants. In Table I there are shown the results obtained by incorporation of various phosphate and halo-hydrocarbon phosphate esters in a base oil comprising 25 approximately 96.5 percent di-isooctyl adipate and 0.5 percent phenothiazine.

TABLE I

Four ball mean  
Hertz load test, kg.

|                                                               |    |
|---------------------------------------------------------------|----|
| Base oil                                                      | 32 |
| Base oil+3% tricresyl phosphate                               | 32 |
| Base oil+3% tri(p-chlorophenyl) phosphate                     | 25 |
| Base oil+3% diphenyl-o-chlorophenyl phosphate                 | 29 |
| Base oil+3% di-( $\beta$ -chloroethyl) 2-ethylhexyl phosphate | 35 |
| Base oil+3% tris(trichloropropyl) phosphate                   | 38 |
| Base oil+3% bis(o-chlorophenyl) phenyl phosphate              | 40 |

The above results indicate that the only three materials which have a sufficiently high mean Hertz load value 40 to merit further consideration are the di-( $\beta$ -chloroethyl) 2-ethylhexyl phosphate and tris-(trichloropropyl) phosphate and the additive of this invention, namely di(o-chlorophenyl) phenyl phosphate. Compounds as closely related to di(o-chlorophenyl) phenyl phosphate as tri(p-chlorophenyl) phosphate and diphenyl-o-chlorophenyl phosphate are much inferior EP agents. Efforts to make the tri(o-chlorophenyl) phosphate not shown in the table were unsuccessful; apparently steric hindrance prevents the formation of tri(o-chlorophenyl) phosphate. The superiority of di(o-chlorophenyl) phenyl phosphate over all the EP and anti-wear agents tested is also significant.

In Table II there are shown the results of subjecting the ester lubricants containing the three EP agents which passed the screening test in Table I in the oxidation-corrosion test of MIL-L-7808B. The base oil was the same used in Table I, namely comprising 96.5 percent di-isooctyl adipate, 0.5 percent phenothiazine; 3% EP agent was used in each test.

TABLE II

| Oxidation-Corrosion Test (347° F./72 Hr.) | MIL-L-7808B Spec. | Di (o-chlorophenyl) phenyl phosphate | Di ( $\beta$ -chloroethyl) 2-ethylhexyl phosphate | Tris-(trichloropropyl) phosphate |
|-------------------------------------------|-------------------|--------------------------------------|---------------------------------------------------|----------------------------------|
| mg./sq. cm.:                              |                   |                                      |                                                   |                                  |
| Cu.....                                   | ±0.4              | 0.0                                  | -2.0                                              | -5.5                             |
| Al.....                                   | ±0.2              | 0.0                                  | +0.2                                              | +0.1                             |
| Mg.....                                   | ±0.2              | 0.0                                  | -4.0                                              | -11.2                            |
| Fe.....                                   | ±0.2              | 0.0                                  | +0.2                                              | +0.1                             |
| Ag.....                                   | ±0.2              | 0.0                                  | +1.2                                              | +0.6                             |

The data in the above table clearly indicate that di( $\beta$ -chloroethyl) 2-ethylhexyl phosphate and tris(trichloropropyl) phosphate degrade the oxidation-corrosion properties of an ester-base lubricant to a serious degree. In contrast, di(o-chlorophenyl) phenyl phosphate completely

meets the rigid requirements of the oxidation-corrosion test of MIL-L-7808B, demonstrating that it alone of all the phosphate and halo-phosphate esters tested provides a high level of EP and anti-wear properties without degrading the oxidation and corrosion properties of ester-type lubricants designed for lubrication of turbo-prop and turbo-jet engines.

The formulation of finished lubricants containing the EP additive of this invention is illustrated in the following examples.

#### Example IV

A blend was prepared having the following composition:

|                                                                             | Percent by weight |
|-----------------------------------------------------------------------------|-------------------|
| 5 Di-2-ethylhexyl sebacate                                                  | 79.5              |
| Polymer of butyl methacrylate in di-2-ethylhexyl sebacate (40% concentrate) | 18.0              |
| Di(o-chlorophenyl) phenyl phosphate                                         | 2.0               |
| Phenothiazine                                                               | 0.5               |

10 The properties of this blend are shown in Table IV.

TABLE III

|                                                                              | MIL-L-7808B<br>Limits | Examples |          |        |
|------------------------------------------------------------------------------|-----------------------|----------|----------|--------|
|                                                                              |                       | I        | II       | III    |
| Flash, COC, °F                                                               | 350 (min.)            | 405      | 410      | 460    |
| Kin. Vis., cs. at:<br>210° F                                                 | 3.0 (min.)            | 4.60     | 4.70     | 7.63   |
| 100° F                                                                       | 11.0 (min.)           | 17.17    | 17.60    | 29.00  |
| -65° F                                                                       | 13,000 (max.)         | 9,374    | 9,684    | 13,164 |
| Viscosity stability (3 hr. at -65° F), percent                               | ±3 (max.)             | +1.9     | +0.4     | +0.3   |
| Pour Point, °F                                                               | -75 (max.)            | -75      | -75      | -75    |
| Foam Test, Seq. 1, 2, 3 ml.                                                  | 100-25-100 max.       | 20-0-0   | 10-10-20 | 0-20-0 |
| Panel Coking Test, 600° F./8 Hrs., mg                                        | 100 (max.)            | 23       | 37       | 49     |
| Evaporation, 400° F/6½ Hrs., percent                                         | 50 (max.)             | 12.1     | 12.9     | 8.3    |
| "H" Rubber Swelling, percent                                                 | 12-35                 | 21.8     | 22.7     | 18.0   |
| Corrosion, 450° F/50 Hr. mg./sq. in.:<br>Copper                              | 3.0 (max.)            | -1.4     | -0.3     | -0.7   |
| Silver                                                                       | 3.0 (max.)            | -0.4     | -0.5     | 0.0    |
| SOD Lead Corrosion, 325° F./1 Hr., Mg./sq. in.                               | 6 (max.)              | 0.2      | -3.2     | -      |
| Corrosion and Oxidation stability, 347° F./72 Hrs., wt. change, mg./sq. cm.: |                       |          |          |        |
| Cu                                                                           | ±0.4                  | -0.4     | 0.0      | 0.0    |
| Al                                                                           | ±0.2                  | 0.0      | 0.0      | 0.0    |
| Mg                                                                           | ±0.2                  | 0.0      | 0.0      | 0.0    |
| Fe                                                                           | ±0.2                  | +0.1     | 0.0      | 0.0    |
| Ag                                                                           | ±0.2                  | 0.0      | 0.0      | 0.0    |
| Vis. Inc., 100° F., percent                                                  | -5 to +15             | +1.6     | 0.91     | 2.8    |
| Total Acid No. Inc.                                                          | 2.0 (max.)            | 0.9      | 0.95     | 0.3    |

#### Example I

A blend was prepared having the following composition:

|                                                                                                                            | Percent by weight | 40 |
|----------------------------------------------------------------------------------------------------------------------------|-------------------|----|
| Di-isoctyl azelate                                                                                                         | 95.3              |    |
| Copolymer of 50% lauryl methacrylate and 50% stearyl methacrylate in a di-2-ethylhexyl sebacate base oil (50% concentrate) | 2.0               |    |
| Di(o-chlorophenyl) phenyl phosphate                                                                                        | 2.0               |    |
| Phenothiazine                                                                                                              | 0.5               |    |
| Disalicylidene 1,2-diaminopropane                                                                                          | 0.2               |    |

The properties of this product are shown in Table III.

#### Example II

A blend was prepared having the following composition:

|                                                                                                                            | Percent by weight | 50 |
|----------------------------------------------------------------------------------------------------------------------------|-------------------|----|
| Di-isoctyl azelate                                                                                                         | 95.5              |    |
| Copolymer of 50% lauryl methacrylate and 50% stearyl methacrylate in a di-2-ethylhexyl sebacate base oil (50% concentrate) | 2.0               |    |
| Di(o-chlorophenyl) phenyl phosphate                                                                                        | 2.0               |    |
| Phenothiazine                                                                                                              | 0.5               |    |

The data in Table III indicate the superior turbine lubricants which are formulated using the extreme pressure additive of this invention. The compositions of Examples I, II and III, meet the rigid requirements of the MIL-L-7808B specification from the standpoints of extreme pressure and wear properties and of oxidation and corrosion resistance.

In Table IV there is shown the properties of the high viscosity composition of Example 4, which was formulated to meet the requirements of a British specification for jet engine lubricants wherein the viscosity requirements are substantially higher than they are in the U. S. military specification.

TABLE IV

|                                                           | Example 4<br>Compositions |
|-----------------------------------------------------------|---------------------------|
| Kin. vis. at:                                             |                           |
| 210° F                                                    | 9.37.                     |
| 100° F                                                    | 39.3.                     |
| -40° F                                                    | 5671.                     |
| -65° F                                                    |                           |
| Pour point                                                | -75.                      |
| Flash                                                     | 430.                      |
| Vis. stab., -65° F                                        |                           |
| Foam test, Sq. 1, 2, 3                                    | 30; 30; 30.               |
| Panel coking test, 600° F./8 hr., mg                      | 29.                       |
| Evap., 400° F./6½ hr., percent                            | 10.3.                     |
| "H" rubber swell, percent                                 |                           |
| Corr. 450° F./50 hr., mg./sq. in.:                        |                           |
| Cu                                                        | -1.1.                     |
| Ag                                                        | -0.3.                     |
| SOD Pb corr                                               |                           |
| Oxidation-corrosion test,<br>347° F./72 hr., mg./sq. cm.: |                           |
| Cu                                                        | +0.0 stain.               |
| Al                                                        | 0.0 stain.                |
| Mg                                                        | 0.1 stain.                |
| Fe                                                        | 0.0 stain.                |
| Ag                                                        | 0.0 stain.                |
| Vis. inc., percent                                        | 1.8.                      |
| Neut. no. inc.                                            | 0.68.                     |

The properties of this blend are shown in Table III.

#### Example III

A blend was prepared having the following composition:

|                                                                                                                                         | Percent by weight | 60   |
|-----------------------------------------------------------------------------------------------------------------------------------------|-------------------|------|
| Di-2-ethylhexyl sebacate                                                                                                                | percent by weight | 91.5 |
| Methacrylate copolymer of 50% lauryl methacrylate and 50% stearyl methacrylate in a di-2-ethylhexyl sebacate base oil (50% concentrate) | percent by weight | 6.0  |
| Di(o-chlorophenyl) phenyl phosphate                                                                                                     | do                | 2.0  |
| Phenothiazine                                                                                                                           | do                | 0.5  |
| Kerosine concentrate of 10 weight percent dimethyl silicone                                                                             | p. p. m.          | 150  |

The properties of this blend are shown in Table III.

75

The high viscosity product, whose properties are shown in Table IV, meets the extreme pressure, wear and oxidation-corrosion requirements of MIL-L-7808B. It is noteworthy that di(o-chlorophenyl) phenyl phosphate is effective as an EP and anti-wear agent in a wide variety of ester base lubricants.

Obviously, many modifications and variation of the invention, as hereinbefore set forth, may be made without departing from the spirit and scope thereof and, therefore, only such limitations should be imposed as are indicated in the appended claims.

We claim:

1. A lubricant composition of matter consisting essentially of an aliphatic carboxylic acid ester of lubricating oil characteristics and di(o-chlorophenyl) phenyl phosphate in an amount sufficient to impart EP and anti-wear properties to said composition.

2. A lubricant composition according to claim 1 in which said ester is an aliphatic diester of an aliphatic dicarboxylic acid containing at least 6 carbon atoms.

3. A lubricant composition according to claim 1 containing 0.2 to 5 weight percent of di(o-chlorophenyl) phenyl phosphate.

4. A lubricant composition consisting essentially of an aliphatic di-carboxylic acid ester of lubricating oil characteristics, 0.2 to 5 weight percent di(o-chlorophenyl) phenyl phosphate, an oxidation inhibiting amount of phenothiazine and a methacrylate polymer in a V. I. improving amount.

5. A lubricant composition according to claim 4 con-

taining between 1.0 to 3.0 weight percent di(o-chlorophenyl) phenyl phosphate, 0.1 to 1.5 percent phenothiazine, and 1.5 to 8 weight percent methacrylate polymer.

6. A lubricant composition according to claim 4 in which the major component is a dioctyl sebacate.

7. A lubricant composition according to claim 4 in which the major component is a dioctyl azelate.

8. A lubricant composition according to claim 4 in which the major component is a dioctyl adipate.

9. A lubricant composition consisting essentially of a dialiphatic ester of an organic dicarboxylic acid, said ester having lubricating characteristics, 1 to 3 weight percent di(o-chlorophenyl) phenyl phosphate, 0.1 to 1.5 percent phenothiazine, 1.5 to 8 weight percent methacrylate polymer, and 0.05 to 0.6 weight percent disalicylidene, 1,2-diaminopropane.

#### References Cited in the file of this patent

#### UNITED STATES PATENTS

|           |          |               |
|-----------|----------|---------------|
| 2,006,756 | Bartram  | July 2, 1935  |
| 2,282,513 | Downing  | May 12, 1942  |
| 2,529,190 | Rocchini | Nov. 7, 1950  |
| 2,542,604 | Weisel   | Feb. 20, 1951 |

#### OTHER REFERENCES

- "Symposium on Synthetic Lubricants," A. S. T. M. Tech. Pub., No. 77, (1947), page 23.  
 Davey, "The Mechanism of Action of E. P. Agents," Scientific Lubrication, September 1949, pages 7-14.